

# UNITED STATES PATENT OFFICE.

OTTO E. RUHOFF, OF MADISON, WISCONSIN, ASSIGNOR TO FRENCH BATTERY & CARBON CO., OF MADISON, WISCONSIN, A CORPORATION OF WISCONSIN.

## ELECTRIC BATTERY.

1,352,087.

Specification of Letters Patent.

Patented Sept. 7, 1920.

No Drawing.

Application filed November 21, 1918. Serial No. 263,593.

To all whom it may concern:

Be it known that I, OTTO E. RUHOFF, a citizen of the United States, residing at Madison, in the county of Dane and State 5 of Wisconsin, have invented a certain new and useful Improvement in Electric Batteries, of which the following is a specification.

This invention relates to electric batteries, both of the type in which there is a bibulous lining of pulp board or similar material close to the zinc can, and also the other type, in which the depolarizing material is compressed around the carbon pencil, and 15 in which a suitable electrolyte is poured into the space between the core or bobbin and the zinc can.

The object of the invention is to construct such batteries in which the depolarizing 20 material is of such a character that the battery will have a very long life, particularly when kept in storage on the shelves of ordinary merchants vending such batteries, and will be really efficient after such storage. The invention consists in the use of an exceedingly pure manganese compound 25 which has not been heretofore used in electric batteries. It also consists in the features and details which will be hereafter 30 more fully set forth in the specification and claims.

One ingredient of the depolarizing mixture of the battery is commonly some ore of manganese present largely or wholly in 35 some form of dioxid. The common practice in the past has been to use such manganese ores in dry batteries without preliminary treatment other than crushing to a desired degree of fineness. I have found after 40 extensive experimentation that if these managanese ores are subjected to treatment before being used in dry batteries, the resulting product is greatly improved. A preferred method of treatment consists in 45 placing a suitable quantity of the pulverized manganese ore in a suitable stirring apparatus and adding to it enough dilute acid, as for example sulfuric acid, so that the whole mixture when thoroughly stirred is 50 thin enough to flow readily. The strength of the acid used is regulated in such a way that when the treatment is completed, the liquid still contains free acid to the extent of about 3% to 6% or more. The acid or 55 other solvent material used must be one that, while it will act strongly enough on

the impurities so as to remove them, will not attack and destroy to any appreciable extent the manganese dioxid compound contained in the ore.

After the manganese ore has been sufficiently treated with dilute acid, with or without the application of heat, the liquid portion of the mixture is removed by any suitable means; as for example, by filtration 65 and washing. After this operation, the purified manganese ore may be dried partly or wholly as desired. It has also been found that in applying this kind of treatment, it may be desirable to add carbonaceous material, such as calcined petroleum coke, in order that the final material, after drying, will be of a rather loose consistency rather than being caked into lumps so hard that difficulty is found in reducing the dried 70 material to a suitably pulverized condition.

By treatment as described, it is possible to remove from manganese ores certain impurities, such as minerals containing copper, arsenic, nickel, cobalt, cadmium, antimony, and the like, hereafter referred to as "poisonous metals". The treatment described need not necessarily remove all of the poisonous metals referred to. In fact, 100% removal is unnecessary. What is required is the removal of such minerals or such parts of harmful minerals as would later on become soluble in the battery electrolyte and would thus diffuse to the zinc container of the battery, where they would 80 be deposited out and set up a local chemical action resulting in a deterioration of the battery, even when the battery is standing 90 entirely idle.

Material prepared by the above process, 95 which is satisfactory for use in a dry battery, should be able to stand the following test: When leached with ordinary battery electrolyte as commonly used in the art, the same being approximately a 30% zinc chlorid 100 solution saturated with sal ammoniac, it will give no indication of such poisonous material. The manganese material which will stand such test is then taken and used in forming the depolarizing material of an electric battery. One such battery which has given satisfactory results contains 50 parts of the prepared manganese, 49 parts of carbonaceous material, 10 parts of sal ammoniac and 12 parts of a zinc chlorid, 45° Baumé 110 solution.

Actual tests of such a battery in which the

manganese compound used is that of the old art; *i. e.*, which has not been prepared to stand the above test show the following results:—

5 *Batteries containing manganese ore as received.*

|    | Sample number of manganese ore used. | Amperage when fresh. | Amperage after 1 year's storage. | Drop in amperage. | Percent drop in amperage. |
|----|--------------------------------------|----------------------|----------------------------------|-------------------|---------------------------|
| 10 | 1168                                 | 36                   | 10                               | 26                | 72.2                      |
|    | 1169                                 | 38                   | 10                               | 28                | 73.7                      |
|    | 1170                                 | 38                   | 13                               | 25                | 65.8                      |
|    | 1171                                 | 39                   | 17                               | 22                | 56.4                      |
|    | 1137                                 | 35                   | 17                               | 18                | 51.4                      |
|    | 1133                                 | 42                   | 16                               | 26                | 61.9                      |
|    | 1131                                 | 37                   | 13                               | 24                | 64.9                      |

On the other hand, tests of such a battery containing the purified manganese of this invention, show the following results:—

20 *Batteries containing same manganese ore, purified.*

| 25 |      |    |    |    |      |
|----|------|----|----|----|------|
|    | 1168 | 37 | 28 | 9  | 24.3 |
|    | 1169 | 36 | 26 | 10 | 27.8 |
|    | 1170 | 37 | 27 | 10 | 27.0 |
|    | 1171 | 37 | 26 | 11 | 29.9 |
|    | 1137 | 34 | 29 | 5  | 14.7 |
|    | 1133 | 39 | 29 | 10 | 25.6 |
|    | 1131 | 41 | 28 | 13 | 31.7 |

30 From a comparison of the two above tables, it will be seen that the drop in amperage in the first set of batteries is from two to three times that of the second, which indicates 35 greatly reduced efficiency in the batteries of the old art as compared with those of this invention.

As indicated above, the solvent used must be one which will act so strongly on the impurities as to remove them, but will not attack and destroy, to any appreciable extent,

the manganese dioxide compound contained in the ore. In the appended claims the expression "solvent treated manganese ore" is to be understood as applying to an ore which 45 has been treated with a solvent which serves to substantially eliminate the poisonous impurities, without unduly attacking the manganese dioxide compound. It may be stated, also, that the treatment has a tendency to 50 increase the porosity of the ore and thus confer upon it a property which is beneficial for battery purposes.

Having thus described my invention, what I claim as new and desire to secure by Letters 55 Patent, is:—

1. An electric battery using a depolarizing material, one of whose elements is a solvent-treated manganese ore of such a character that when leached with a 30% zinc chlorid 60 solution saturated with sal ammoniac, substantially no trace of poisonous metals is shown.

2. An electric battery, combining with the usual positive and negative elements, a depolarizing mixture comprising 50 parts of manganese dioxide compound, 49 parts carbonaceous materials, 10 parts sal ammoniac, and 12 parts of a zinc chlorid 45° Baumé solution, the manganese dioxide used being of 70 such a character that when leached with a 30% zinc chlorid solution, saturated with sal ammoniac, substantially no trace of poisonous metal is shown.

In witness whereof, I have hereunto subscribed my name in the presence of two witnesses.

OTTO E. RUHOFF.

Witnesses:

BEN W. PARK,  
MABEL S. NELSON.